

# UNITED STATES PATENT OFFICE.

CHARLES M. STINE, OF WILMINGTON, DELAWARE, ASSIGNOR TO E. I. DU PONT DE NEMOURS AND COMPANY, OF WILMINGTON, DELAWARE, A CORPORATION OF DELAWARE.

## PROCESS OF MAKING EXPLOSIVE COMPOUNDS AND PRODUCT THEREOF.

1,370,067.

Specification of Letters Patent.

Patented Mar. 1, 1921.

No Drawing.

Application filed May 31, 1917. Serial No. 171,980.

To all whom it may concern:

Be it known that I, CHARLES M. STINE, of Wilmington, in the county of New Castle, and in the State of Delaware, have invented a certain new and useful Improvement in Processes of Making Explosive Compounds and Product Thereof, and do hereby declare that the following is a full, clear, and exact description thereof.

10 My invention relates particularly to a process for producing explosives of an advantageous character, and the product thereof. The object of my invention is to provide a process for producing explosives and particularly explosive compounds containing a nitro group and nitrate groups, or a plurality of nitro groups and nitrate groups, and the product produced thereby. A further object of my invention is to provide compounds of this character in which a nitro group is located in the ring of a molecule of an aromatic compound and a plurality of nitrate groups are located in one side chain of the compound.

25 While my invention is capable of embodiment in many different forms, for the purpose of illustration I have described only certain forms thereof. For example, I may proceed as follows:

30 The compound produced in accordance with my process may be, for example, any one of the following:

- 35  $C_6H_5(CH(NO_2)_2CH_2(NO_2)_2)(NO_2)_2$   
 $C_6H_2CH_2(CH(NO_2)_2CH_2NO_2)_2(NO_2)_2$   
 $C_6H_2CH_2NO_2(CH(NO_2)_2CH_2NO_2)_2(NO_2)_2$   
 $C_6H_2(CH(CH_2NO_2)_2)_2(NO_2)_2$   
40  $C_6H_2OH(CH_2NO_2)_2(NO_2)_2$   
 $C_6H_2(CH_2NO_2)_2CH_2NO_2$   
 $C_6H_2CH_2(CH_2NO_2)_2(NO_2)_2$

In carrying out my process a hydrocarbon of the benzene series and having a side chain consisting of an alkyl with a plural carbon nucleus, as for example, methyl-ethyl-benzene, may be chlorinated at varying temperatures, the flow of chlorin being continued until a theoretical increase in weight has been attained corresponding to 45 the chlor derivative desired. The chlorination is carried out in such way that chlorin becomes attached to each of the primary and secondary carbon atoms of the side chain. The chlorinated compound is then

nitrated preferably in the ordinary way by applying a mixture of nitric and sulfuric acids according to the procedure usually followed in nitration, preferably until the dinitro compound is obtained. The nitrated material is heated with pure water, 60 preferably under a pressure of about 20 pounds per square inch, until the chlorine atoms in the side chain have been replaced by hydroxyl groups.

The aqueous solution is then evaporated 65 to drive off the water and hydrochloric acid, and the dinitrophenyl compound is nitrated further according to the well known method by the application of a mixture of sulfuric and nitric acids, resulting in substituting a nitrate group for each hydroxyl group in a side chain. The material thus obtained, which can be separated from the spent acid, or which may be obtained by drowning the spent acids with 70 subsequent separation, is, after drying, suitable for use as an explosive or an ingredient in explosives. The explosive thus obtained is exceedingly powerful and quite 75 stable.

Such compounds may also be prepared by other processes, as, for example, a nitration of an aromatic hydrocarbon containing at least one side chain to the mono-, di-, or tri-nitro compound, chlorination of the 80 dinitro compounds to cause chlorin to become attached to carbon atoms of the side chain, hydrolysis of the chlor-nitro compound to produce a nitro hydroxyl compound and nitration of the nitro-hydroxyl 85 compound to produce a nitro nitrate.

While I have described my invention above in detail, I wish it to be understood that many changes may be made therein without departing from the spirit of my invention. For example, I do not wish to limit myself to any particular method of preparation, and I wish it to be understood that the compounds produced in accordance 90 with my invention may be used as such or in mixtures of various kinds, as desired.

I claim:

1. A process of producing an explosive compound which comprises nitrating and halogenating an aromatic compound which 105 contains a side chain comprising an alkyl with a plural carbon nucleus so as to introduce a nitro group into the molecule and

a plurality of halogen atoms into the side chain, hydrolyzing to substitute hydroxyl groups for the halogens, and nitrating to substitute nitrate groups for the hydroxyl groups.

2. A process of producing an explosive compound which comprises nitrating and halogenating a benzenoid hydrocarbon which contains a side chain comprising an alkyl with a plural carbon nucleus so as to introduce a nitro group into the molecule and a plurality of halogen atoms in the side chain, hydrolyzing to substitute hydroxyl groups for the halogens, and nitrating to substitute nitrate groups for the hydroxyl groups.

3. A process of producing an explosive compound which comprises nitrating and halogenating a hydrocarbon of the aromatic series which contains a side chain comprising an alkyl with a plural carbon nucleus so as to introduce a nitro group into the molecule and a plurality of halogen atoms into the side chain, hydrolyzing to substitute hydroxyl groups for the halogens, and nitrating to substitute nitrate groups for the hydroxyl groups.

4. A process of producing an explosive compound which comprises nitrating and halogenating a hydrocarbon of the aromatic series which contains a side chain comprising an alkyl with a plural carbon nucleus so as to introduce a plurality of nitro groups into the ring and a plurality of halogen atoms into the side chain, hydrolyzing to substitute hydroxyl groups for the halogens, and nitrating to substitute nitrate groups for the hydroxyl groups.

5. A process of producing an explosive compound which comprises nitrating and halogenating ethyl benzol so as to introduce a nitro group into the ring and a plurality of halogen atoms into the side chain, hydrolyzing to substitute hydroxyl groups for the halogens, and nitrating to substitute nitrate groups for the hydroxyl groups.

6. A process of producing an explosive compound which comprises nitrating and halogenating ethyl benzol so as to introduce a plurality of nitro groups into the ring and a plurality of halogen atoms into the side chain, hydrolyzing to substitute hydroxyl groups for the halogens, and nitrating to substitute nitrate groups for the hydroxyl groups.

7. A process of producing an explosive compound which comprises nitrating and halogenating an aromatic compound which contains a side chain comprising an alkyl with a plural carbon nucleus so as to introduce a nitro group into the molecule and a plurality of halogen atoms into the side chain, hydrolyzing to substitute hydroxyl groups for the halogens, and nitrating to substitute nitrate groups for the hydroxyl

groups, the halogenation being carried out before the initial nitration.

8. A process of producing an explosive compound which comprises nitrating and halogenating a hydrocarbon of the aromatic series which contains a side chain comprising an alkyl with a plural carbon nucleus so as to introduce a nitro group into the molecule and a plurality of halogen atoms into the side chain, hydrolyzing to substitute hydroxyl groups for the halogens, and nitrating to substitute nitrate groups for the hydroxyl groups, the halogenation being carried out before the initial nitration.

9. A process of producing an explosive compound which comprises nitrating and halogenating an aromatic compound which contains a side chain comprising an alkyl with a plural carbon nucleus so as to introduce a plurality of nitro groups into the molecule and a plurality of halogen atoms into the side chain, hydrolyzing to substitute hydroxyl groups for the halogens, and nitrating to substitute nitrate groups for the hydroxyl groups, the halogenation being carried out before the initial nitration.

10. A process of producing an explosive compound which comprises nitrating and halogenating a hydrocarbon of the aromatic series which contains a side chain comprising an alkyl with a plural carbon nucleus so as to introduce a plurality of nitro groups into the ring and a plurality of halogen atoms into the side chain, hydrolyzing to substitute hydroxyl groups for the halogens, and nitrating to substitute nitrate groups for the hydroxyl groups, the halogenation being carried out before the initial nitration.

11. A process of producing an explosive compound which comprises nitrating and halogenating ethyl benzol so as to introduce a nitro group into the ring and a plurality of halogen atoms into the side chain, hydrolyzing to substitute hydroxyl groups for the halogens, and nitrating to substitute nitrate groups for the hydroxyl groups, the halogenation being carried out before the initial nitration.

12. A process of producing an explosive compound which comprises nitrating and halogenating ethyl benzol so as to introduce a plurality of nitro groups into the ring and a plurality of halogen atoms into the side chain, hydrolyzing to substitute hydroxyl groups for the halogens, and nitrating to substitute nitrate groups for the hydroxyl groups, the halogenation being carried out before the initial nitration.

13. An explosive comprising an organic compound of the aromatic series having a side chain, said compound containing a nitro group and having a plurality of nitrate groups in the side chain.

14. An explosive comprising an organic

compound of the aromatic series having a side chain and containing a plurality of nitro groups and having a plurality of nitrate groups in the side chain.

5 15. A composition containing an organic compound of the aromatic series having a side chain, said compound containing a nitro group and having a plurality of nitrate groups in the side chain.

10 16. A composition containing an organic compound of the aromatic series having a side chain and containing a plurality of

nitro groups and having a plurality of nitrate groups in the side chain.

17. An organic compound of the aromatic 15 series having the formula:—



In testimony that I claim the foregoing I have hereunto set my hand.

CHARLES M. STINE.

Witnesses:

E. K. BOLTON,  
P. E. STRICKLAND.